

## UNITED STATES PATENT OFFICE

2,196,153

PROCESS OF REGENERATING FUSED  
SALTPETER BATHS

Josef Martin Michel, Bitterfeld, Germany, assignor to I. G. Farbenindustrie Aktiengesellschaft, Frankfort-on-the-Main, Germany

No Drawing. Application April 12, 1938, Serial  
No. 201,639. In Germany April 27, 1937

2 Claims. (Cl. 252—5)

This invention relates to a process of regenerating fused saltpeter baths which have, in the course of their employment, become partially decomposed.

5 Fused alkali metal nitrates (i. e. potassium or sodium nitrate) or mixtures thereof are frequently employed in the heat-treatment of alloys, particularly aluminium alloys, as a means for heating the metal to or maintaining it at certain temperatures in a reliable and easily controllable manner. It has now however been ascertained that a partial progressive decomposition of such fused nitrate baths occurs in the course of usage, such decomposition at first only 10 yielding nitrite and oxygen; the nitrite formed then gradually further decomposes so as to ultimately yield free alkali. The free oxygen formed by decomposition is apt to react with the surfaces of the metal to be treated as well as 15 with any exposed metallic surface of the containers of the baths, whilst the free alkali formed by further decomposition, in turn, is capable of reacting with such metal oxides, with formation, e. g. of alkaline reacting aluminates and ferrites, 20 which become dissolved in the saline melt. This attack of the decomposition products present in the "degenerated" saline baths of the kind referred to, upon exposed metallic surfaces, is particularly strong in the temperature range 25 at which the baths are generally employed (about 200—500° C.).

The present invention aims at regenerating such "degenerated" fused nitrate baths. This is achieved, according to the invention, by adding 30 to the salt melts such amounts of alkali metal dichromate as are sufficient to convert the alkali metal oxides or other alkaline reaction compounds resulting from the decomposition, and also any alkali metal nitrite formed in the first 35 stage of decomposition into monochromate, for example in accordance with the equations:

- (1)  $K_2Cr_2O_7 + 2KOH = 2K_2CrO_4 + H_2O$
- (2)  $2Na_2AlO_3 + 3Na_2Cr_2O_7 = Al_2O_3 + 6Na_2CrO_4$
- (3)  $2K_2FeO_3 + 3K_2Cr_2O_7 = Fe_2O_3 + 6K_2CrO_4$
- (4)  $K_2Cr_2O_7 + 2KNO_2 = N_2O_3 + 2K_2CrO_4$

It has moreover been ascertained that, on addition of di-chromate, the reactions represented by the foregoing Equations 1 to 4 proceed with 40 different speed in the saltpeter melt, the reactions occurring in accordance with Equations 1 to 3 supra, being completed in a relatively short time (after a few hours), while the reaction with nitrite sets in substantially only after reactions 45 1 to 3 have been completed and only becomes

complete after a few days, when all the nitrite originally present in the "degenerated" bath has become decomposed.

The presence of the monochromate thus formed in the bath substantially prevents the further decomposition of the latter owing to the existence of equilibria between alkali metal nitrate, alkali metal nitrite and alkali metal monochromate, in which the proportion of alkali metal nitrite is extremely small. 5

The required amount of alkali metal dichromate (to be calculated on the basis of the foregoing Equations 1 to 4) may either be added all at once to the "degenerated" melt, or else the amounts determined from Equations 1 to 3 may 10 first be added and, after neutralisation has taken place, the portions required for the reaction with the nitrite present are added. 15

The regeneration of the bath by addition of 20 bichromate is preferably effected at temperatures between about 300 and 350° C., since at higher temperatures the reactions occurring as a result of the addition of bichromate may assume an explosive character. 25

## Example

To a "degenerated" saltpeter melt originally consisting of a mixture of equal parts of potassium nitrate and sodium nitrate and containing, as the products of decomposition of the 30 original bath, according to analysis, 1.9% by weight of nitrite (calculated as  $N_2O_3$ ) in addition of 0.3% by weight of alkaline reacting components

$$\left( \text{calculated as } \frac{K_2O}{2} + \frac{Na_2O}{2} \right)$$

35 the amount of dichromate required to neutralise, with formation of monochromate, the alkalinity of the bath, was first added. After two hours the melt, according to a test made, had become completely neutralised. Thereupon, the amount of dichromate calculated as being necessary to decompose the alkali metal nitrite, was added. In 40 the course of a few days the  $N_2O_3$  value of the bath was then observed to vary as follows: 45

| Time                   | Percent of $N_2O_3$ |
|------------------------|---------------------|
| Initial condition..... | 1.91                |
| After 24 hours.....    | 1.18                |
| After 48 hours.....    | 0.68                |
| After 72 hours.....    | 0.27                |
| After 96 hours.....    | 0.16                |

50 55 After four days the melt contained practically

no more nitrite and was thus completely regenerated.

I claim:

5 1. A process of regenerating fused saltpeter baths, for the heat-treatment of alloys, which have degenerated in the course of use with the formation of decomposition products comprising free alkali, alkali metal aluminates or ferrites, alkali metal nitrite, which comprises adding to such fused anhydrous baths at a temperature not substantially exceeding about 350° C. an alkali metal dichromate in the amount required to con-

vert such decomposition products into monochromate.

10 2. Process in accordance with claim 1, in which at first only such amounts of dichromate are added to the baths as are necessary to neutralise the alkalinity of the baths, and after neutralisation has taken place, a further quantity of dichromate sufficient to decompose the nitrite present, with formation of monochromate, is added.

JOSEF MARTIN MICHEL.